

# UNITED STATES PATENT OFFICE.

WILLIAM D. PARDOE, OF TRENTON, NEW JERSEY, ASSIGNOR TO THERMOID RUBBER COMPANY, OF HAMILTON TOWNSHIP, TRENTON, NEW JERSEY, A CORPORATION OF NEW JERSEY.

## BRAKE-LINING AND METHOD FOR PREPARING THE SAME.

1,277,108.

Specification of Letters Patent. Patented Aug. 27, 1918.

No Drawing.

Application filed March 16, 1917. Serial No. 155,330.

To all whom it may concern:

Be it known that I, WILLIAM D. PARDOE, a citizen of the United States, and a resident of Trenton, Mercer county, State of New Jersey, have invented Brake-Linings and Methods for Preparing the Same, of which the following is a specification.

One object of my invention is to provide an improved lining for clutches, brakes and the like which shall be capable of withstanding stresses placed upon it under operating conditions, shall possess good wearing surface and be of such a nature as not likely to be damaged by overheating.

In carrying out my invention I provide a solution which in a typical case may consist of twenty-six ounces of asphalt, four ounces of red lead, five ounces of sulfur, two ounces of hexamethylenetetramin in two

thousand eight hundred and forty c. c. of gasolene and three hundred and fifty c. c. of benzol. The woven or braided cloth or tape to be treated, which may be made of flax, hemp, asbestos or other fibrous material, is placed in this solution for a time sufficient to permit it to be completely impregnated or saturated, after which it is removed from the solution, thoroughly dried, and subjected to a relatively high pressure such as fifteen hundred pounds to the square inch, being at the same time heated to a temperature of from 300° to 400° F.

As a result of this treatment the materials in the fabric are vulcanized to a greater or less extent and the quantity of fixed carbon therein is materially increased, so that the finished product has an unusually high coefficient of friction, possesses good wearing qualities, and will not become sticky when subjected to the heat to which it is frequently exposed under operating conditions. Moreover the finished product produced as above described is hard, unaffected by oil and heat, and is as nearly uninflammable as it is possible to make. It is noted that the substance referred to above as asphalt is preferably the mineral compound known as gilsonite, in an oxidized or "blown" form, although other hydrocarbons of an asphaltic nature may be employed without departing from my invention.

The hexamethylenetetramin is employed to accelerate the vulcanization of the ma-

terials with which the fabric base is impregnated and while it may be replaced by other substances which hasten oxidation or vulcanization, I prefer to employ it or some other amin. Obviously other lead oxids besides red lead might be used but I have found the latter to give the best results. Again, some solvent other than a mixture of gasolene and benzol may be used for dissolving the materials specified, such for example as carbon bisulfid or carbon tetrachlorid, but I preferably utilize the substances specified.

It is to be noted that the lead oxid and hexamethylenetetramin may be altogether omitted in some cases although I have found them to be particularly valuable in materially hastening the vulcanizing or oxidizing operation.

I claim:—

1. The method of making a brake lining which consists in passing a body of fabric through a solution containing asphalt, an oxid of lead, sulfur, and an oxidation accelerator; and thereafter treating said fabric to vulcanize the material with which it is impregnated.

2. The method of making a brake lining which consists in passing a body of fabric through a solution containing asphalt; an oxid of lead, sulfur, and an oxidation accelerator; and thereafter subjecting said fabric to a relatively high pressure and temperature to vulcanize the material with which it is impregnated.

3. The method which consists in impregnating a fabric with asphalt; an oxid of lead, sulfur and an oxidation accelerator; and thereafter treating said fabric to vulcanize the substances with which it is impregnated.

4. The method which consists in impregnating a body of fabric with asphalt, lead oxid, sulfur and an amin; and thereafter subjecting said fabric to a vulcanizing treatment.

5. The method which consists in impregnating a body of fabric with asphalt, a lead oxid, sulfur and hexamethylenetetramin; and thereafter subjecting said fabric to a vulcanizing process.

6. The method which consists in passing a body of fabric through a solution containing asphalt and sulfur to impregnate the

same therewith; and thereafter subjecting said fabric to a vulcanizing process.

7. A brake lining consisting of a body of fibrous material impregnated with the substance resulting from the vulcanization of a mixture of asphalt, a metallic oxid and sulfur.

8. A brake lining consisting of a body of fibrous material impregnated with the product of the vulcanization of asphalt, red lead and sulfur.

9. A brake lining consisting of a highly compressed body of fabric uniformly impregnated with the product of the vulcanization of asphalt, red lead and sulfur.

10. A brake lining consisting of a highly compressed body of fabric uniformly im-

pregnated with the product resulting from the vulcanization of asphalt and sulfur.

11. The method of making a brake lining 20 which consists in impregnating a body of fabric with asphalt and an oxidation accelerator; and thereafter subjecting said fabric to a relatively high pressure and temperature.

12. A brake lining consisting of a highly compressed body of fabric uniformly impregnated with the product resulting from the exposure of asphalt and a vulcanizing agent to a temperature of from 300° to 30 400° F.

In witness whereof I affix my signature.

WILLIAM D. PARDOE.